

Sept. 6, 1932.

C. H. EGAN ET AL

1,876,450

SELF TIGHTENING CONTAINER CLOSURE

Filed Dec. 17, 1927



Inventors  
Charles H. Egan  
Bradley Dewey  
by Robert Cushman Woodbury.  
Attest.

## UNITED STATES PATENT OFFICE

CHARLES H. EGAN, OF BOSTON, AND BRADLEY DEWEY, OF CAMBRIDGE, MASSACHUSETTS, ASSIGNEES TO DEWEY AND ALMY CHEMICAL COMPANY, OF CAMBRIDGE, MASSACHUSETTS, A CORPORATION OF MASSACHUSETTS

## SELF-TIGHTENING CONTAINER CLOSURE

Application filed December 17, 1927. Serial No. 240,756.

Our invention relates to closures for containers, and is characterized by a novel and useful relationship between the container-members (e. g., vessel and cover) which in juxtaposition provide confining walls of a seam-space, and the material confined in such seam-space as a sealing or "caulking" material.

The efficiency of a container closure is conditioned by the relationship of the sealing material to the contents of the container. If the contents consist of or comprise a material which is sufficiently fluid to insinuate itself into the sealed seam, and which acts upon the sealing material in the seam to disintegrate the same, loss of sealing efficiency is only a question of time. Many containers, such as cans, are sold without knowledge on the part of their maker of the materials which will be stored in them; if, for instance, the sealing material provided be immune to water but not to oils, and the cans be used to contain oily material, the final result will be unsatisfactory.

Our invention herein described, is concerned with the relationship of colloidal mutual extension as between the more or less fluid contents of a container and the seal substances, and with means for controlling the effects of such mutual extension. The seal substances are in substantially solid condition in the seal. If, of several ingredients in the container closure seal, confined closely in a sealing seam, one at least is unsusceptible of gel formation with the fluid contents of the container, its presence, cooperating with the physical confinement of the seal material by the container-members, will check and control the progress of other component or components toward sol formation, if one or more of such be susceptible of gel and sol formation with the said contents. Thus, a container closure depending on rubber as a cardinal ingredient, while reliable and durable to hold can contents comprising water or the common alcohols or ketones, will deteriorate if the container is filled with material containing oils, or typical solvents of rubber such as benzol, naphtha, carbon tetrachloride, etc., whereas some sealing materials

which are susceptible to water or the common alcohols or ketones would retain can contents comprising ingredients which attack rubber. As a very large proportion of materials habitually stored in sealed containers have either a water or an oil base, it is desirable to furnish a container closure which is, by its composition, inherently able to resist or compensate for the deteriorating action of such contents.

The drawing hereto annexed illustrates, in much enlarged cross section, the seam joint between a can and its head. In this drawing, B represents part of the can body, T part of the can top, and S a sealing composition, originally deposited in an annular peripheral channel of the can top, and tightly confined between the two container-members in the seam formed by double-rolling the edges thereof together, in the manner shown. Such containers constitute probably the most conspicuous example of containers comprising closely juxtaposed body and cover members, forming a confined seam-space for the retention of sealing material; other and analogous examples are furnished by bottle caps and the like, held to the container by pressure.

Further exemplification of our invention is as follows: Attach to one of the members of a container, either the body or cover, a sealing material, containing approximately equal quantities of rubber, and either or both of the other following named materials:

(1) A rubber, which is insoluble, in, or not forming a gel with, water, or with alcohols or ketones.

(2) A substance insoluble in, or not forming a gel with, oils, or common rubber solvents or with alcohols or ketones.

(3) A substance insoluble in, or not forming a gel with, common alcohols or ketones, or with rubber solvents.

This may be done by applying such a mixture, preferably suspended or dissolved in a menstruum in the usual manner as by filling an annular seam-groove in a can head, or by painting on the flange of a can. In case the compound is solid or too viscous to flow at ordinary temperatures, it may be heated. However, as a rule the compound is a liquid with

the oil (or common rubber solvent) unsusceptible, and/or common alcohol (or ketone) unsusceptible, and the rubber components dissolved or dispersed therein, and the composition thus deposited is dried, and the container closure is then ready for the sealing operation.

It is obvious that the amount of fluid which can be applied is limited by the size of the 10 annular groove in the can head. As a result, to obtain an efficient seal, the percentage of solid matter must be reasonably high. We have found that fillers aid by increasing the 15 percentage of solid matter, are unaffected by most solvents, increase the plasticity of the mass after attack by a solvent, and also function as "wicks" to facilitate drying, thus avoiding blistering.

Sometimes it is convenient to add softeners 20 such as glycerin, invert sugars, diethylene glycol, etc., which keep the dried seals from becoming brittle.

The container closure, completed by attachment of the body and cover, as by double-seaming a can head to a can body, or by evacuating a jar and fixing a cover thereon by atmospheric pressure or otherwise, tightly confines the above-described sealing material in the seal joint, and so long as the sealing material remains tightly confined in said joint, the contents of the can or other container will be adequately protected. If the canner uses cans or containers thus sealed to hold materials comprising an oil, the oil-susceptible rubber particles contained in the seal, when selectively attacked by the contents, start to swell, be attacked, that is, to form a gel, or dissolve; but the oil-unsusceptible ingredient, intimately associated with the oil-susceptible ingredient, being unsusceptible to the can contents, retards and eventually restrains the swelling or solution, and prevents the swelling or solution action from extruding the seal material from the space within which the closure confines it. If the same container is used for material having a water base, the water-unsusceptible rubber ingredient functions as the restraining factor and prevents the initial alteration of the water-susceptible ingredient from proceeding to a degree damaging to the integrity of the seal as a whole. The restrained swelling action, in either case, operates to tighten the 55 sealing material in the container closure, so that the container closure is self-tightening in either emergency. If with rubber there be compounded a material which forms a gel with alcohol or a ketone, with which rubber 60 does not form a gel, the closure which comprises within its seam-walls such a composition with rubber will be self-tightening in the presence of alcohol or ketone contents of the container, the rubber acting as the sustaining factor when the alcohol or ketone gel-

forming constituent starts to swell and disintegrate.

And likewise, if with rubber there be compounded a water-gel former and an alcohol-gel former, either rubber solvents, water, or alcohol, etc., may be safely placed in the container, since the restraining factor is provided for each alternative.

When using water as the initial vehicle, we prefer to make these compounds by making a 75 solution, with or without heat, of the water-soluble ingredient, in a portion of the water to be used. Preservatives may be added during this solution. We then make an artificial dispersion, if a natural dispersion is not used, of the insoluble ingredient in the balance of the water, by grinding it in a pebble mill or in one of the ordinary types of colloid mills with water, and, if desired, one or more protective colloids together with such alkaline or acid bodies as may aid to stabilize the resultant suspension. The solution and the dispersion, together with any desired fillers and softeners, are then mixed by stirring, 80 with or without heat. If desired, the fillers may be mixed with the insoluble constituent before grinding. Our invention may be visualized by considering that where oil is brought into contact with rubber or other similar colloids, the first thing to happen is 85 an absorption of the oil by such colloids, and that when water is brought into contact with solid glue or other similar colloids, the first thing to happen is an absorption of the water by such colloids. The absorption in either case continues until a very marked swelling has taken place, until which time there is no 90 solution of the rubber-like products into the oil or of the glue-like products into the water. These properties are both well recognized, and 95 our invention consists in utilizing them so that as the masses of the affected ingredient swell they are held tightly confined between the walls of the container by the ingredient which is unaffected by the solvent in such a 100 way that the solvents can not get at them sufficiently to have their full disintegrating effect. In other words, due to the homogeneous and mutually distributed condition of the mixture and the space between the walls in 105 which it is confined, the colloidal network of the unaffected ingredient holds back and prevents the washing away of the other ingredient which is being attacked by the contents of the container. This action is reinforced and made even more effective because 110 of the fact that as the solvent penetrates the sealing material the attacked ingredients swell and are thereby even more firmly bound within the network and within the confined space between the walls. Thus in coaction with the confinement by the seam space walls this swelling tightens the seal and makes 115 it much more difficult for the contents of the container to get through from the interior of 120

- the container and attack further the sealing material. The relative proportions of the mutually distributed rubber-like and glue-like ingredients may be varied, but it is absolutely necessary to have in the sealing material an effectively substantial proportion of each ingredient. A preferred mixture is one having rubber and glue in approximately the same proportions, and the following are examples of good workable formulae for sealing material which will confer self-tightening capacity upon the container closure.
- (1) Bentonite 2 parts, gum karaya 0.4 part, sodium fluoride 0.15 part, water, including that of the rubber latex, 81.75 parts, sodium carbonate 0.24 part, ammonia 1 part, animal glue 7.23 parts, rubber, as rubber latex, 7.23 parts.
- (2) Bentonite 2 parts, gum karaya 0.4 part, sodium fluoride 0.15 part, water, including that of the rubber latex, 78.85 parts, sodium carbonate 0.24 part, ammonia 1 part, glycerin 2.9 parts, animal glue 7.23 parts, rubber, as rubber latex, 7.23 parts.
- (3) Bentonite 2 parts, gum karaya 0.4 part, sodium fluoride 0.15 part, water, including that of the rubber latex, 73.04 parts, sodium carbonate 0.24 part, ammonia 1 part, glycerin 2.9 parts, animal glue 7.23 parts, rubber, as rubber latex, 7.23 parts, whiting 5.81 parts.
- In the above-scheduled examples of self-tightening sealing compounds, the glue in (1), (2), and (3) exemplifies the water-gel forming, or water-soluble factor; the latex-rubber in (1), (2) and (3), exemplifies the oil- or common rubber solvent-gel-forming factor.
- The other ingredients named are supplemental; bentonite, karaya gum with sodium carbonate, ammonia for alkaline reaction constitute as a group a filling, dispersion-stabilizing factor; whiting is a convenient filler; sodium fluoride is a preservative; glycerin a softener.
- It will be evident to those skilled in the art that these are but samples of mixtures that will provide a self-tightening closure such as has been described, and that the essential feature is the use with rubber of a constituent unaffected by rubber solvents but susceptible to solvents to which rubber is indifferent. For the sake of brevity, we prefer to describe these constituents as constituents capable or incapable of gel formation, irrespective of whether the attack or solvent action tends to form a gel within the narrow meaning of the word; i. e. if it forms a colloidal solution.
- We claim:
1. A sealed container comprising a sealed joint including spaced walls and a sealing material confined between said walls, said sealing material comprising, in its operative condition, a substantially homogeneous mixture including rubber and a substance capable of gel formation with water, the rubber and gel forming substance being in such substantial proportions that each, while in confinement between said walls, shall furnish effective restraint against substantial removal of the other by substances which are normally capable of accomplishing such removal.
2. A sealed container comprising a sealed joint including spaced walls and a sealing material confined between said walls, said sealing material comprising, in its operative condition, a substantially homogeneous mixture including rubber and glue, the rubber and glue being in such relative proportions that each, while in confinement between said walls, shall furnish effective restraint against substantial removal of the other by substances which are normally capable of accomplishing such removal.
3. A container comprising a sealed joint including spaced walls and a sealing material confined between said walls, said material, when in operative condition between said walls, being substantially homogeneous in structural consistency and including rubber and a substance capable of gel formation with water, the rubber and gel forming substance being in approximately equal proportions.
- Signed by us at Cambridge, Massachusetts, this 14th day of December 1927.
- CHARLES H. EGAN.  
BRADLEY DEWEY.